

L. D. DAVIS.  
MANUFACTURE OF SEAMLESS TUBES.  
APPLICATION FILED OCT. 22, 1912. RENEWED OCT. 8, 1914.  
**1,123,178.** Patented Dec. 29, 1914.

FIG.1.



FIG.2.



WITNESSES:

J. Herbert Bradley  
Thos. B. Joyce

INVENTOR  
Leonard D. Davis  
by Dennis S. Wolcott  
Atty

# UNITED STATES PATENT OFFICE.

LEONARD D. DAVIS, OF ERIE, PENNSYLVANIA.

## MANUFACTURE OF SEAMLESS TUBES.

1,123,178

Specification of Letters Patent.

Patented Dec. 29, 1914.

Application filed October 22, 1912, Serial No. 727,208. Renewed October 8, 1914. Serial No. 865,776.

To all whom it may concern:

Be it known that I, LEONARD D. DAVIS, residing at Erie, in the county of Erie and State of Pennsylvania, a citizen of the United States, have invented or discovered certain new and useful Improvements in Manufacture of Seamless Tubes, of which improvements the following is a specification.

10 The invention described herein relates to an improved method of manufacturing seamless tubes from hollow billets and has for its object the application of reducing pressure in such manner, that while there will always be sufficient transverse movement of metal to prevent any detrimental gripping of the mandrel by the billet, the displacement due to the applied pressure will be almost wholly substantially parallel 20 to the axis of the billet and there will be relatively little resistance to this longitudinal flow of the metal.

It is well known to blacksmiths and hammer men, that if a flow of metal in a particular direction is desired, the area of contact of one of the reducing surfaces, (as the fuller) with the metal must be less in the desired direction of flow than in any other direction.

30 It will be readily understood that if the wall of a metal tube is reduced by hammering or pressing it upon an interior round bar or mandrel, such mandrel itself tends to act somewhat like a fuller to expand the tube transversely if the external pressure is applied by a relatively large or flat face making an area of contact which is of greater extent lengthwise of the mandrel than crosswise, because the metal can more readily flow crosswise. Very similarly, in 40 rolling plates or sheets between a pair of cylindrical rolls, the flow of the metal is almost entirely at right angles to the roll axes. If in the case of a tube upon a mandrel, instead of a relatively flat external reducing face, a fuller having an edge concave crosswise of the tube and narrow in the direction lengthwise of the mandrel be applied to reduce the tube, the metal displaced by the edge of the fuller will flow laterally of that edge and therefore lengthwise of the mandrel with comparative freedom, whereas the relatively great extent of contact of the edge of the fuller crosswise 50 of the mandrel and the consequent confin-

ing of the metal thereby against the mandrel tend to prevent any substantial flow of metal circumferentially. These considerations will aid in understanding the present invention.

Heretofore in reducing billets by cross rolling in the Mannesmann method, the extent of contact of the metal on the rolls and mandrel has been such that greater longitudinal than circumferential resistance is 65 offered to the flow of metal. Under such conditions the greater flow is circumferential and to produce material elongation, the metal must crowd its way forward and spirally around the mandrel and is thereby subjected to great and injurious stress.

70 In the accompanying drawings forming a part of this specification, Figure 1 is a side elevation of the parts or elements of a machine immediately operative on the metal in the practice of my improved method, and Fig. 2 is a sectional plan view of another form of apparatus adapted to carry out said method.

75 In the practice of my invention reduction of the billet is effected by the conjoint action of convex interior and concave exterior surfaces, the latter operating obliquely on the billet and moving in planes at an angle to the axis of the billet.

80 My improved method can be carried out by several forms or constructions of apparatus, as for example by the form shown and described herein or by the form of apparatus forming the subject-matter of an application Serial No. 709,014, filed by me July 12, 1912, wherein apparatus is claimed.

85 In the construction shown in Fig. 1, the exteriorly acting reducing members consist of a plurality of rings or annular members 1 90 suitably supported as for example in circular housings as shown in the application referred to. The housings are so constructed and arranged that the plane of rotation of the reducing rings will be so inclined to the 100 axis of the billet as to impart to the latter a longitudinal movement. The rings are so mounted eccentrically as regards the axis of the billet that the points of least eccentricity or the points at which the inner surfaces of 105 the rings contact with the billet are equally spaced around and equally spaced along the line of longitudinal movement of the billet, so that each ring will not only serve as a reducing element, but will also operate to sup- 110

port the billet while being acted on by the other rings. Additional supports for the billet while being reduced are provided by any suitable means, such as a plurality of 5 rings 2, so mounted as to be capable of rotation, preferably by frictional contact with the billet. These supporting rings are so arranged that their oblique rolling actions and planes of rotation will have substantially 10 the same inclination to the axis of the billet as the reducing rings in order that the longitudinal movement of the billet may not be retarded. The rings 1 have external gear teeth, as shown, for driving them, and have narrow and rounded rolling faces, as shown 15 by the cross-section.

In reducing metal tubes by cross rolls which are convex transversely of the billet, the pressure is applied at an acute angle, instead of perpendicularly, to the surface of 20 the metal at the point where the roll impinges on the metal, thus driving the metal along before the roll in a transverse direction. The greater the convexity of the roll, 25 the more acute will be this angle of applied pressure where the roll first impinges on the metal; and, in any case, where the extent of contact is smaller at right angles to the axis 30 of the billet than longitudinally thereof, displacement will be in the rolling direction transversely of the billet. For reasons hereinbefore stated displacement of metal in the Mannesmann method is spirally around the billet.

35 In my improved method employing an interior convex and an exterior concave surface, if the radius of curvature of the concave surface be as nearly as practicable the same as the radius of the outer surface of 40 the billet, the area of contact between the concave surface and the billet is very large circumferentially and the angle between the approaching reducing surface and billet surface as they come into contact is so small 45 that the impingement is very easy and gradual, and the action of the reducing surface on the metal closely resembles the application of pressure radially in a continuous progression around the billet.

50 When reducing hollow billets by convex cross rolls as in the Mannesmann method, the extent of contact of the rolls on the metal is much greater lengthwise of the billet than it is transversely hence there is great resistance to any longitudinal movement of the metal. This objectionable retardation and 55 in some cases actual prevention of direct longitudinal flow, cannot be overcome when using rolls of a width capable of practical use. By properly proportioning the curvature of a concave surface to the external diameter of the billet the transverse extent of contact of the surface with the billet can be made substantially equal to and in some 60 cases greater than one fourth of the circum-

ference of the billet. As for example in reducing a billet having an external diameter of four inches, the concave reducing surface can be made to have a contact transverse of the billet equal to or greater than three 70 inches. Then by making the reducing portion of the concave surface with a transverse width of about two inches and slightly oval or with rounded edges there will be less resistance to longitudinal movement of the 75 metal than to its transverse movement. In other words in the practice of my improved method, reducing pressure is so applied to the billet that displacement of metal will produce elongation and very little transverse displacement. While it is preferred 80 that the concave surface should have its extent of contact greater transversely than longitudinally such relative proportioning of the extent of contact is not necessary to 85 getting some advantage from concave rolls, as when using a concave reducing surface as described, there will be less resistance to longitudinal movement of the metal than with any other forms of reducing surface, 90 even if the preferred relative proportioning of the contact surface be varied.

In lieu of employing a series of longitudinally spaced rings as shown in Fig. 1, a construction requiring the employment of a 95 stiff mandrel for small thin tubes, the method described herein can be carried out by the form of apparatus shown in Fig. 2, and forming the subject-matter of an application filed November 29, 1912, and patented 100 July 22, 1913, No. 1,067,806, to E. S. Diescher. This mill consists of two substantially annular housings 4, provided with bearings 5 for the annular hubs 6 of the disks 7. These disks are formed with central openings, the walls of which are shaped to form annular reducing surfaces *a*, which however may be formed on rings 8, secured in seats on the disks. The housings are arranged in such relation to each other that the axes of the rings are out of alinement, so that the line of movement X—X of the billet and mandrel through the rings forms an acute angle with the axes of the rings. The reducing surfaces *a* are formed on such an 115 angle with reference to the axes of the rings as to form a converging-mouthed pass for the billet. It will be observed in the figure that the rings are not parallel, but slightly inclined oppositely to each other transversely to the section plane of the drawing, so that the cross rolling action will be correspondingly oblique on the billet, and, as shown in the section, the rolling faces are 120 substantially narrow and convex so as to 125 make narrow contact longitudinally of the pass. It will be observed that the reducing surface of one ring when operative on the billet is diametrically opposite the reducing surface of the other ring. The peripheries 130

of the disks 7 are toothed to intermesh with pinions 9 on the shafts 10, whereby the disks are rotated in their bearings.

Great difficulty is experienced in the practice of the Mannesmann method in preventing undue transverse enlargement of the tube. This is due to the reasons explained and the fact that the lines of pressure of convex surfaces on the billet except on the lines passing through the axes of the rolls and billet are diverging and hence the reducing pressures force the metal transversely, thereby expanding it away from the mandrel. Even when disks are used to reduce the billets the lines of pressure will diverge from a line passing through the axis of the billet and the points where the surfaces of the disks are nearest the center of the billet.

It is characteristic of my improved method involving the employment of convex and concave reducing surfaces that pressure is so applied that the line of the external pressure through any one point of contact of the concave surface will converge in the direction of the billet toward lines through any other points of contact of that surface in the same plane transverse of the billet. Hence in my improved method the concave surface will have slight tendency to cause material enlargement of the internal diameter of the billet.

I claim herein as my invention:

1. As an improvement in the art of making seamless tubes, the method of cross-rolling which consists in subjecting the tubular billet to oblique cross-rolling and pressure between an internal mandrel and an external cross-rolling surface which is narrow lengthwise of the tube and is concave in the oblique cross-rolling plane, applying the external rolling pressure over a contact area which is relatively narrow lengthwise

of the tube and relatively wide circumferentially, and thereby simultaneously elongating and advancing the tube. 45

2. As an improvement in the art of making seamless tubes, the method of cross-rolling which consists in subjecting the tubular billet to oblique cross-rolling and pressure by an external cross-rolling surface which is concave in the plane of its oblique cross-rolling motion, applying the pressure over a contact area which is relatively narrow lengthwise of the tube and 55 relatively wide circumferentially, and thereby simultaneously elongating and advancing the tube.

3. As an improvement in the art of making seamless tubes, the method of cross-rolling which consists in subjecting the tubular billet to cross-rolling and pressure between an internal mandrel and an external cross-rolling surface which is convex and narrow lengthwise of the mandrel and 65 concave in the plane of its cross-rolling motion, and thereby simultaneously decreasing the wall thickness and elongating the tube.

4. As an improvement in the art of making seamless tubes, the method of cross-rolling which consists in subjecting the tubular billet to oblique cross-rolling and pressure between an internal mandrel and an external concave cross-rolling surface which is concave in the plane of the oblique cross-rolling motion and restricting the external pressure to a contact area on the tubular billet which is relatively narrow lengthwise of the mandrel and extensive circumferentially of the mandrel. 75 80

In testimony whereof, I have hereunto set my hand.

LEONARD D. DAVIS.

Witnesses:

PHIL J. SMITH,  
S. H. DROWN.